

## UNITED STATES PATENT OFFICE

2,381,127

## LUBRICATING COMPOSITION

Lebbeus C. Kemp, Jr., Scarsdale, N. Y., assignor  
to The Texas Company, New York, N. Y., a cor-  
poration of Delaware

No Drawing. Application February 25, 1943,  
Serial No. 477,135

18 Claims. (Cl. 252—48)

The present invention relates to lubricating compositions possessing extreme pressure properties, and particularly to an additive composition which, when incorporated in lubricating oils and greases, imparts extreme pressure properties thereto.

The additive ingredients of the present invention are prepared from the phenolic compositions present in or derived from the oils extracted from the *Anacardium* genus of the *Anacardiaceae* family. The oils included within this classification are such oils as cashew nut shell oil, marking nut shell oil, Japanese lac, etc., whose chemical composition depends upon the particular method of extraction used. It is the consensus of the authorities on these extracted oils that the chemical composition of the naturally-occurring oils consists primarily of various types of aromatic derivatives such as anacardic acid ( $C_{22}H_{32}O_3$ ), cardol ( $C_{32}H_{52}O_4$ ), cardanol ( $C_{20}H_{32}O$ ), anacardol ( $C_{18}H_{30}O$ ), urushiol ( $C_{20}H_{30}O_2$ ), etc. These aromatic derivatives are very unstable and in the presence of heat form decomposition products or oil-insoluble polymerization products.

Representative of these naturally-occurring oils is cashew nut shell oil which, when obtained by solvent extraction, consists primarily of 90% anacardic acid and 10% cardol. The anacardic acid portion of this solvent-extracted oil, which is described as a salicylic acid homolog, decomposes at slightly elevated temperatures with the evolution of carbon dioxide to yield cardanol, which is a phenol containing an unsaturated alkyl radical ( $C_{14}H_{27}$ ) in the meta position. This decomposition is particularly noticed in the cashew nut shell oil obtained by a thermal extraction process which contains only about 16% anacardic acid, with the balance made up of a major proportion of cardanol and a minor proportion of cardol.

It has been found that an ester of phosphoric acid in which the ester radical is derived from the unsaturated alkyl phenols obtained from an oil extracted from the *Anacardium* genus of the *Anacardiaceae* family which have been modified by the presence of one or more substituent groups in the unsaturated alkyl radicals, is possessed of exceptional extreme pressure properties when incorporated in a hydrocarbon oil. These ester radicals are preferably those obtained from the aforementioned unsaturated alkyl phenols which contain either sulfur or a halogen such as chlorine or mixtures thereof in the unsaturated alkyl radicals. In accordance with the present invention a high pressure lubricant is obtained by the addition of small quantities of these phosphoric acid esters to a suitable lubricating oil or grease base. As examples of these high pressure lubricants may be mentioned gear lubricants, gear oils, cutting oils, pressure greases, lubricating oils for internal combustion engines, etc.

These extreme pressure additives are prepared from the oil-soluble unsaturated alkyl phenols present in or derived from the extracted oils and may take the form of mono-di- or tri-esters of phosphoric acid, with preference given to the tri-ester. Examples of the unsaturated alkyl phenols suitable for the preparation of these additives are cardanol, anacardol, urushiol, and the oil-soluble phenolic components which have not been isolated and which may be present in admixture with other phenols in the distillate and distillate residues of the extracted oils. These unsaturated alkyl phenols are relatively unstable and susceptible to polymerization and condensation reactions in the presence of acids and elevated temperatures. This instability may be overcome by partially hydrogenating the unsaturated constituents prior to the preparation of the substituted derivatives forming a part of the present invention, or by a choice of substitution reactions which will avoid polymerization. The stabilization of the unsaturated alkyl phenols is not critical to the preparation of the phosphoric acid esters and as such is not intended as a limitation to the products of the present invention.

The phosphoric acid esters may be incorporated in a hydrocarbon oil, and particularly in mineral lubricating oils and greases in amounts ranging between 0.1-10.0% by weight, depending upon the type of hydrocarbon oil base and the degree of extreme pressure properties desired. The particular range of proportions as applied to some of the lubricating oils and grease bases may be outlined as follows:

|                      | Per cent by weight of finished lubricant |
|----------------------|------------------------------------------|
| Gear lubricants      | 0.5 - 5.0                                |
| Gear oils            | 0.5 - 5.0                                |
| Cutting oils         | 0.5 - 3.0                                |
| Motor oils           | 0.25 - 1.5                               |
| Aircraft engine oils | 0.5 - 2.0                                |
| Diesel oils          | 0.5 - 2.0                                |
| Turbine oils         | 0.1 - 0.5                                |

In the preparation of the substituted unsaturated alkyl phenols and the phosphoric acid esters thereof, any of the classical methods of synthesis may be used. The particular methods chosen depend upon the conditions of reaction and the stability of the phenolic compositions. When preparing the sulfur and/or halogenated derivatives of the unsaturated alkyl phenols it is preferable to select a method of preparation which is carried out at low temperatures and which does not yield acidic by-products or where the acidic by-products are removed from the reaction zone. These conditions of reaction, however, may be modified if the starting material has been stabilized by partial hydrogenation.

The phosphoric acid esters of the substituted derivatives may be prepared by any of the gen-

erally accepted methods of preparation since the product resulting from the substitution reactions is sufficiently stable in and of itself to be reacted under normal conditions.

When preparing the halogenated derivatives and particularly a chlorinated derivative, of the unsaturated alkyl phenols, the phenolic composition is preferably subjected to partial hydrogenation. The partially hydrogenated product may then be dissolved in an inert solvent such as ethylene dichloride or tetrachlorethane, and chlorine gas or dry hydrogen chloride gas passed in until a weight increase corresponding to 1 or 2 mols is obtained. The chlorinated derivative is then washed free of excess halide and the solvent removed. When it is desired to obtain a mixed sulfur-chlorine derivative, sulfur monochloride may be used in place of the chlorine or hydrogen chloride previously mentioned.

In preparing the sulfurized or sulfur-containing derivatives the phenolic composition may either be partially hydrogenated or reacted in its full unsaturated condition, depending upon the methods of incorporating sulfur.

The following example of the preparation of a tri-ester of phosphoric acid, in which the ester radical was derived from partially hydrogenated sulfurized cardanol obtained from cashew nut shell oil, is given as an illustration of one of the methods of preparing these phosphoric acid esters:

*Example*

400 ccs. (370-380 grams) of freshly distilled cardanol with a bromine no. of 118 was charged to an Adkins type bomb, together with 10-15 grams of Raney nickel. Hydrogen was admitted to 2000-2200 pounds per square inch and the bomb rocked at 250-300° F. until the pressure dropped to 1000-1100 pounds per square inch. The process was repeated until a quantity of hydrogen had been added sufficient to give a calculated bromine no. of 85-95. In this particular case the resulting bromine no. was 95. After hydrogenation the product was filtered free of Raney nickel. 400 grams of the partially hydrogenated cardanol were then sulfurized with 28 grams of sulfur at 330-350° F., which was calculated to give a sulfur content in the product of from 5 to 7%. The resulting partially hydrogenated sulfurized cardanol was then dissolved in toluene and 115 grams of pyridine were added. To this solution was then added 80 grams of  $\text{POCl}_3$  at room temperature. The reaction mixture was allowed to stand for 16 hours and was thereafter stirred at 65-75° C. for an additional four hours. The phosphate ester was then filtered free of pyridine hydrochloride and the solvent removed by stripping. The analysis of the tri-phosphate ester of partially hydrogenated sulfurized cardanol was as follows:

|                         | Found | Theory. |
|-------------------------|-------|---------|
| Percent phosphorus..... | 2.4   | 2.3     |
| Percent sulfur.....     | 6.3   | 6.9     |

The effectiveness of the phosphoric acid esters of the present invention as extreme pressure agents when incorporated in lubricating oils has been demonstrated by tests conducted on an Almen testing machine. For these tests the product obtained by the foregoing example was incorporated in a solvent-refined, dewaxed, Mid-Continent lubricating oil of an S. A. E. 30 grade. The

results obtained (indicated as the pounds of pressure required for seizure) were as follows:

|                                                                                  | Pounds<br>5-10 |
|----------------------------------------------------------------------------------|----------------|
| Reference oil.....                                                               |                |
| Reference oil + 1% partially hydrogenated sulfurized tri-cardanyl phosphate..... | 134.7          |

(\* Represents average of 6 test runs.)

Obviously many modifications and variations of the invention as hereinbefore set forth may be made without departing from the spirit and scope thereof, and therefore only such limitations should be imposed as are indicated in the appended claims.

15 I claim:

1. A lubricant comprising a hydrocarbon oil containing 0.1-10.0% by weight of a substituted alkyl phenyl ester of phosphoric acid, said substituted alkyl phenyl ester being derived from the unsaturated alkyl phenols present in or derived from the oils extracted from the *Anacardium* genus of the *Anacardiaceae* family and characterized by the presence of at least one substituent group selected from the class consisting of sulfur and halogen in the unsaturated alkyl radicals thereof.

2. A lubricant comprising a mineral lubricating oil containing 0.1-10.0% by weight of a substituted alkyl phenyl ester of phosphoric acid, said substituted alkyl phenyl ester being derived from the unsaturated alkyl phenols present in or derived from the oils extracted from the *Anacardium* genus of the *Anacardiaceae* family which have been modified by the addition of substituent groups selected from the class consisting of sulfur and halogen in the unsaturated alkyl radicals thereof.

3. A lubricant comprising a major proportion of a hydrocarbon oil and a minor proportion, sufficient to impart extreme pressure properties to said hydrocarbon oil, of a substituted alkyl phenyl ester of phosphoric acid, said substituted alkyl phenyl ester being derived from the unsaturated alkyl phenols present in or derived from the oils extracted from the *Anacardium* genus of the *Anacardiaceae* family which have been modified by the addition of substituent groups in the unsaturated alkyl radicals thereof, said substituent groups being selected from the class consisting of sulfur and a halogen.

4. A lubricant comprising a hydrocarbon oil containing 0.1-10.0% by weight of a substituted alkyl phenyl ester of phosphoric acid, said substituted alkyl phenyl ester being derived from the unsaturated alkyl phenols present in or derived from cashew nut shell oil which have been modified by the addition of substituent groups selected from the class consisting of sulfur and halogen in the unsaturated alkyl radicals thereof.

5. A lubricant comprising a mineral lubricating oil containing 0.1-10.0% by weight of a substituted alkyl phenyl ester of phosphoric acid, said substituted alkyl phenyl ester being derived from the unsaturated alkyl phenols present in or derived from cashew nut shell oil which have been modified by the addition of substituent groups selected from the class consisting of sulfur and halogen in the unsaturated alkyl radicals thereof.

6. A high pressure lubricant comprising lubricating oils and greases having incorporated therein 0.1-10.0% by weight of a substituted alkyl phenyl ester of phosphoric acid, said substituted alkyl phenyl ester being derived from the unsaturated alkyl phenols present in or de-

70

rived from the oils extracted from the Anacardium genus of the Anacardiaceae family, and characterized by the addition of at least one substituent group selected from the class consisting of sulfur and halogen in the unsaturated alkyl radicals thereof.

7. A lubricant comprising a mineral lubricating oil containing 0.1-10.0% by weight of a substituted tri-alkylphenyl ester of phosphoric acid, said substituted tri-alkylphenyl ester being derived from the unsaturated alkyl phenols present in or derived from oils extracted from the Anacardium genus of the Anacardiaceae family which have been modified by the addition of substituent groups selected from the class consisting of sulfur and halogen in the unsaturated alkyl radicals thereof.

8. A lubricant comprising a mineral lubricating oil containing 0.1-10.0% by weight of a substituted tri-alkylphenyl ester of phosphoric acid, said substituted tri-alkylphenyl ester being derived from unsaturated alkyl phenols present in or derived from cashew nut shell oil which have been modified by the addition of substituent groups in the unsaturated alkyl radicals thereof.

9. A high pressure lubricant comprising lubricating oils and greases having incorporated therein 0.1-10.0% by weight of a substituted alkyl phenyl ester of phosphoric acid, said substituted alkyl phenyl ester being derived from the unsaturated alkyl phenols present in or derived from cashew nut shell oil, and characterized by the addition of at least one substituent group selected from the class consisting of sulfur and halogen in the unsaturated alkyl radicals thereof.

10. A lubricant comprising a hydrocarbon oil containing 0.1-10.0% by weight of a substituted alkyl phenyl ester of phosphoric acid, said substituted alkyl phenyl ester being derived from the partially hydrogenated unsaturated alkyl phenols present in or derived from cashew nut shell oil and characterized by the addition of at least one substituent group selected from the class consisting of sulfur and halogen in the unsaturated alkyl radicals thereof.

11. A lubricant comprising a hydrocarbon oil and 0.1-10.0% by weight of sulfurized tri-cardanyl phosphate.

12. A lubricant comprising a mineral lubricating oil and 0.1-10.0% by weight of sulfurized tri-cardanyl phosphate.

13. A lubricant comprising a hydrocarbon oil and 0.1-10.0% by weight of partially hydrogenated sulfurized tri-cardanyl phosphate.

14. A high pressure lubricant comprising lubricating oils and greases having incorporated therein 0.1-10.0% by weight of partially hydrogenated sulfurized tri-cardanyl phosphate.

15. A lubricant comprising a hydrocarbon oil containing a small quantity, sufficient to impart extreme pressure properties to said hydrocarbon oil, of a substituted alkyl phenyl ester of phosphoric acid, said substituted alkyl phenyl ester being derived from the unsaturated alkyl phenols present in or derived from cashew nut shell oil which have been partially hydrogenated and modified by the addition of sulfur to the remaining unsaturated linkages of the alkyl radical thereof.

16. A lubricant comprising a hydrocarbon oil containing a small quantity, sufficient to impart extreme pressure properties to said hydrocarbon oil, of a substituted alkyl phenyl ester of phosphoric acid, said substituted alkyl phenyl ester being derived from the unsaturated alkyl phenols present in or derived from cashew nut shell oil which have been partially hydrogenated and modified by the addition of chlorine to the remaining unsaturated linkages of the alkyl radical thereof.

17. A lubricant comprising a hydrocarbon oil containing a small quantity, sufficient to impart extreme pressure properties to said hydrocarbon oil, of said substituted alkyl phenyl ester of phosphoric acid, said substituted alkyl phenyl ester being derived from the unsaturated alkyl phenols present in or derived from cashew nut shell oil which have been modified by the addition of sulfur to the unsaturated linkages of the alkyl radical thereof.

18. A lubricant comprising a hydrocarbon oil containing a small quantity, sufficient to impart extreme pressure properties to said hydrocarbon oil, of a substituted alkyl phenyl ester of phosphoric acid, said substituted alkyl phenyl ester being derived from the unsaturated alkyl phenols present in or derived from cashew nut shell oil which have been modified by the addition of chlorine to the unsaturated linkages of the alkyl radical thereof.

LEBBEUS C. KEMP, JR.